

Nov. 14, 1939.

P. H. PENNELL

2,179,562

METHOD OF COATING WEBS

Filed July 24, 1936



## UNITED STATES PATENT OFFICE

2,179,562

## METHOD OF COATING WEBS

Philip H. Pennell, Manheim Township, Lancaster County, Pa., assignor to Armstrong Cork Company, Lancaster, Pa., a corporation of Pennsylvania

Application July 24, 1936, Serial No. 92,295

11 Claims.

(Cl. 91—70)

My invention relates to a method of coating webs and is directed particularly to a method for use in printing floor or other surface coverings requiring a film of paint of appreciable thickness 5 to serve as a wear surface. In the manufacture of printed coverings of this class, there are a number of factors which at the present time militate against the observance of certain fundamental criteria, known to the skilled paint 10 technician as being essential to the formation of a high quality wearing surface from the four most essential standpoints, namely, abrasion resistance, acid and alkali resistance, smoothness and planeness of surface, and finished gloss. 15 These factors arise by reason of the unusually heavy film of paint which must be applied in a single application in order to be economically practicable, and by the fact that curing or stoving of the film must be effected to properly condition the film for use as a wear surface. This necessitates that the base, which is generally in the form of a continuous web, with its applied 20 coating paint, must, at some time almost immediately after application of the paint film, assume an inclined or vertical position. These problems, which are inherent in the application of a heavy film of slow drying paint and in the stoving thereof, are amplified when the curing is effected in the "festoon stoves" commonly employed in the floor covering industry, wherein the material, as it emerges from the printing machine, is directed into a curing chamber and hung 25 therein in vertically extending festoons on cylindrical battens, the length of the festoon generally being in the order of forty-five feet, although similar problems are present when flat rack stoving is utilized. In such operation, the material must assume a substantially vertical position while being directed from the bed of the machine 30 to those racks which lie above or below the plane of the bed, and paint runs are as common in flat rack stoving as in festoon stoving.

Contrary to one of the fundamental prerequisites of satisfactory wear film formation, it has been common practice in the printed floor covering industry to "body up" the paint to prevent paint runs. This has been effected by incorporating relatively large amounts of pigments or other filling agents into the paint. It has been 45 the theory that in such paints the reduction of flowability is due to increased interfacial frictional resistance built up by the pigment particles within the film. In some instances the proportion of pigment has been as high as 44% by 50 volume of the nonvolatile portion of the paint,

whereas it has long been known that the ideal pigmentation for wear films should be approximately 30% by volume of the nonvolatile portion of the paint. Any increase in pigmentation inevitably results in lowering of the wear, alkali 5 and acid resistance of the formed film. An equally acute problem is encountered with "bodied up" paints where the covering material is printed in design. The paint film which is formed by printing with paints having high pigment concentrations will not level out satisfactorily after application but "stands proud", taking the outline of the printing member which applied the film and leaving relatively sharp ribs or ridges where contiguous color patches abut. 10 This condition is aggravated by the use of peg or line block printing members of the type commonly utilized in the printing of floor coverings to provide air relief. Another disadvantage arising out of the use of high pigment concentra- 15 tion paints, lies in the difficulty of obtaining a glossy surface. Gloss is imparted to the surface of the film primarily by the vehicle overlying or surrounding the pigment particles and disposed at the surface of the film. If the pigment concentra- 20 tion is too high, there is insufficient vehicle to adequately wet and coat the pigment particles and, as a result, the dried film is dull and has no appreciable sheen. In addition, the cost of the paint is increased proportionately 25 with any increase in proportion of pigment to vehicle.

The use of "bodied up" paints has minimized paint runs but has not eliminated them completely since the pigment particles will, by their 30 gravitational forces, tend to orient themselves readily upon reduction of viscosity of the vehicle induced by heat, and, the material being subjected to such heat while in a vertical plane, the tendency still remains for the particles to 35 gravitate downwardly, thus forming regions of thick and thin films. While the print paints heretofore employed have possessed some thixotropic body inherent in pigmented vehicle structures, movement of the material through a vertical path has been effected so soon after the printing step, which applies shearing forces to the paint and thus reduces the viscosity thereof, that any material thickening by thixotropic action 45 cannot be availed of prior to movement of the material into the stoves or curing racks, for, under ordinary temperature conditions, such thixotropic action is so slow that it would require 50 a commercially impracticable time period be- 55

tween printing and stoving to avail of such action.

It is an object of my invention to provide a method and means whereby low pigment paints, in the order of 30% concentration, may be used in printing floor coverings or other surfaces requiring a relatively heavy film and may be hung in festoon type stoves or otherwise cured without running. The fact that the material will pass through or remain in a vertical plane for an extended period of time does not materially affect the film when employing the method and apparatus of my invention.

Another object of my invention is to provide a mechanism and method whereby leveling of a film of thixotropic body paint which may be of the usual character and high pigment concentration may be accomplished and paint runs eliminated.

According to a preferred embodiment of my invention, the former object is attained by the use of a vehicle having the characteristic of attaining a false body within the applied film by micelle formation within a relatively short period of time, which micelle formation may be accelerated by the application of heat, and heating the film while maintained in a horizontal plane to reduce the viscosity of the vehicle to thus enhance micelle formation, with consequent thickening and stiffening of the film to a degree sufficient to permit hanging in a festoon, or movement in a vertical plane, substantially immediately after completion of the printing operation and to induce leveling of the applied film into a smooth, plane surface. Leveling, which is dependent upon and results from reduction of the surface tension of the applied film, and gravitational forces, should be accomplished before the creation of the "false body" has proceeded too far, since, if the film is rendered stiff and viscous, leveling, without mechanical working of the film, cannot be accomplished. The false body preferably results from the formation of micelles within the vehicle due to the presence of gel particles and/or resinoid particles therein, and, where the film is pigmented, the pigments may be so chosen that micelle formation is enhanced thereby. The paint thus formed will be in a thixotropic state and will permit of application by the printing machines commonly employed in the floor covering industry.

It is preferred to create the false body effect but temporarily in order that gloss will not be sacrificed and to insure proper cohesion of the film to the surface to which it is applied. For that reason, the resinoid particles should preferably be soluble in the oil of the vehicle, although they may be only difficultly so, in order that the resinoid particles will not be present as such in the final, cured film. The false bodying, resulting in immediate but temporary stiffening of the film, will be replaced by permanent setting or coagulation of the vehicle and conversion of the various components of the film into a stable, tough, flexible, alkali-resistant wear surface.

A typical example of a vehicle of the preferred type may comprise a partially regenerated oil gel, a prepared resinoid, and, if desired, a heat bodied oil gel.

The partially regenerated oil gel may be formed in the following manner: A batch consisting of 2000 pounds of a linseed, China-wood oil mixture is heated in an open kettle to about 565° F. and maintained at that temperature until a semi-solid condition is obtained which may be determined

by examination for a heavy string on a test paddle immersed in the oil immediately after thorough stirring. The oil is then in such condition that continued heating for a short period of time would result in complete solidification of the oil mixture. In order to arrest this action, at least temporarily, a paste comprising a mixture of about 20 pounds of litharge and sufficient oil to produce the proper consistency is incorporated into the batch by stirring. The incorporation of this material results in a regeneration of the gel formed by heating. There is some saponification of the oil structure and, upon incorporation of the litharge, accomplished by stirring, the oils become of flowable consistency but would normally revert to a solid gel upon cooling. Therefore, immediately after sufficient regenerating agent such as litharge has been incorporated, the batch is thinned with a compatible oil. In the example referred to, approximately 1950 pounds of raw linseed oil are added; the material being incorporated slowly and with constant stirring in order to preserve the regenerated gel particles. The product thus formed should have a viscosity of about 4.35 poises at 570° F. and contain a fairly large proportion of suspensoids in the form of gel particles thoroughly dispersed throughout the raw oil and the liquid portion of the oil gel resulting from regeneration thereof. Manganese resinate or other suitable drier in the amount of about three pounds is added, and the batch is permitted to cool to room temperature.

A resinoid which is but difficultly soluble in the above regenerated oil gel may be formed in the following manner: A mixture composed of 35 amberol F-7 and amberol K-12-A and consisting of about 285 pounds of the former resin and 15 pounds of the latter is melted with 114 pounds of regenerated oil gel prepared as above described. The K-12-A amberol is less readily soluble in the regenerated oil gel than the F-7 and the proportions may be varied over a relatively wide range depending upon the amount and rate of micelle formation desired. The temperature of the batch is raised to about 420° F. and maintained at that temperature until the melt is clear. Thereafter the temperature is rapidly raised to about 550° F. It is desirable to first dissolve the resin in the oil under relatively low temperature conditions in order to prevent charring of the resin in the bottom of the heating kettle which might result if the temperature were too high, and thereafter, elevate the temperature of the batch to obtain the desired consistency. The temperature is then reduced to approximately 450° F., accompanied by continuous stirring. Manganese resinate in the amount of about 3/4 of a pound is then added. Thereafter, mineral spirits or other thinning agent are added in the amount of 414 pounds. It is preferred to use a thinning agent in which the resinoid is difficultly soluble, since micelle formation is increased in the final product when a thinner of that type is employed, since by the use of such a thinner the resinoid is broken down into a form in which the particles are capable of rapid micelle formation and are dispersed in the final product in a metastable condition rather than disposed in solution in the thinner. I have obtained satisfactory results, however, when using hydrogenated naphtha which is a fairly good solvent for the amberol resin in the above example. The resinoid is of a flowable consistency and, under ordinary temperature conditions, is not readily soluble in regenerated oil gel of the type above described.

The heat bodied oil gel may take the form of a heat bodied linseed oil formed in the following manner: A batch of approximately 4000 pounds of linseed oil is heated to approximately 500° F. in an open kettle. When this temperature is reached, litharge in the amount of about 14½ pounds is added and stirring effected to properly incorporate this material. The temperature is then elevated to about 590° F. and maintained until a viscosity of approximately 150 poises at 590° F. is attained. A similar batch is made except that the temperature is maintained at 590° F. until a viscosity of 250 poises at 590° F. is attained and thereafter the two batches are blended together. The temperature of the mixture is then permitted to fall to 450° F. and manganese resinate in the amount of about two pounds is added. The product resulting contains a substantial amount of gel which is formed probably by local overheating of the oil in the kettle. In order to maintain a temperature of 590° F., considerable local overheating will occur and this undoubtedly results in the formation of a substantial amount of gel particles. In this heat bodied oil, the litharge is utilized to more rapidly effect gel formation and heat bodying. If the litharge were eliminated, then heat thickening would require a considerably longer period of time and, as a result, the oil would be dark in color and not as satisfactory for some purposes as that prepared in accordance with the preferred procedure.

A typical example of a print paint suitable for use as a wearing surface for floor coverings may be formed by mixing the following ingredients into a paste and then grinding the mixture on a paint mill:

|                     | Pounds |
|---------------------|--------|
| Lithopone           | 38     |
| Zinc oxide          | 25     |
| Whiting             | 37     |
| Regenerated oil gel | 25     |

With 100 pounds of this paste, is mixed, in a suitable paint mixer, 17 pounds of regenerated oil gel, 16 pounds of resinoid, and 4 pounds of heat bodied oil gel.

The resulting paint contains resinoid particles and gel particles formed from both the regenerated oil gel and the heat bodied oil gel. The term "particles" is used in a generic sense, since the resinoid and oil gel particles may be in the form of suspensoids or may be in a colloidal state. The particles are dispersed throughout the vehicle in a metastable condition, and immediately after shearing forces, such as those resulting from the printing operation, cease to be applied, micelle formation begins. This micelle formation is believed to be a direct result of the combined forces of the particles some of which are of an anisotropic character, and gravitational forces. It is probably true that the resinoid and gel particles have some affinity for each other and for themselves and, if the pigment be properly chosen, the particles thereof also will have a tendency to group themselves with the other particles within the film. Coincidentally with micelle formation, there is a general thickening of the applied film. The reaction is not completely understood, but it is believed to result from the fact that with the first formation of micelles, there is immediately an enormous increase in the specific surface of the particles to be wetted and, concomitantly, a diminution in the liquid or vehicle available for wetting. There immediately follows, therefore, a general thick-

ening and stiffening of the whole structure. In order to accelerate this formation, I purpose to apply heat to the paint film disposed upon the surface being coated, while the material rests in a substantially horizontal plane in which running of the applied film will not occur. By the application of heat, the viscosity of the vehicle is reduced and the particles within the paint film are released for proper and immediate orientation. This may be accompanied by vaporization of a portion of the thinner for the resinoid which loss will also have some thickening effect on the film. Since leveling of the paint film is dependent upon the reduction in surface tension and gravitational deposition of the pigment and other particles within the film, it is desirable to apply the heat to the film over an extended period of time, in the order of three minutes, and the temperature should not be so high as to induce micelle formation at too rapid a rate for, as pointed out above, thickening will result before leveling is accomplished. At the present rate of production on flat block printing machines, a heating chamber about 70 feet long would be required for a three minute heating period. This may be objectionable from the standpoint of space limitations, but in many instances the heating chamber may be positioned at a point near the bottom of the curing chamber without any major alterations to existing equipment.

I have found that when a film formed as above described is applied to a foundation web of saturated felt of the type commonly employed in the manufacture of felt base floor covering, a general thickening and stiffening of the applied film and satisfactory leveling may be accomplished if the temperature of the web be elevated to 165° F., and maintained at that temperature for a period of thirty seconds while the material rests in a substantially horizontal plane. By heating to this temperature, a relatively short heating time is necessary. The web may then be immediately transferred to a substantially vertical plane without danger of running.

In the accompanying drawing there is illustrated, in side elevation, a presetting device positioned at the exit end of a flat block printing machine and adapted to properly condition a paint film prior to passage of the web into a curing chamber.

The presetting device 2 is positioned between a flat block printing machine 3 and a curing chamber 4, and is of relatively short length. The exit end 5 of the presetting device may be positioned within the curing chamber 4 as shown. The presetting device comprises a bank of steam coils 6 fed by a header 7 communicating with a suitable source of steam supply. In the embodiment shown, the coils 6 extend transversely of the bed of the printing machine and are secured to supporting framework 8. A second battery of steam coils 9 is disposed in a plane parallel to the bed of the printing machine 3 and these coils are secured between the printing machine frame members 10. The coils 9 are preferably formed of flattened pipes in order to present a relatively flat surface to support the web of decorated material 11 during its travel from the printing machine 3 into the curing chamber 4. It will be observed that the coils 9 lie in a position in advance of the coils 6 in order that the web 11 may be brought to the desired temperature prior to the application of radiant heat to the decorated surface of the web by the coils 6. The coils 9

are provided with a steam inlet 12 feeding into a header 13 to which the coils are connected. A return line 14 is also provided for drainage purposes.

5 The radiating coils 6 and the supporting framework 8 are mounted for movement in a longitudinal direction parallel with the web in order that, upon the filling of the curing chamber, the mechanism may be moved out of the curing 10 chamber and the door D closed. In order to provide a conveniently movable mechanism, end frame members 15 are provided with rollers 16 engageable with tracks 17 attached to the printing machine frame. A roller 18 is secured to 15 the machine frame and engages a track 19 on the supporting framework 8. A supporting roller 20, secured to the framework 8, rides on a track 21 attached to wall 22 of the curing chamber 4. A stop 23 is provided to limit movement of the 20 exit end 5 into the curing chamber.

From the foregoing, it will be clear that after decoration of the web 11 by the printing machine 3 which applies a relatively heavy layer of paint, the web passes over the heating coils 9 whereby 25 the temperature of the web is elevated. The material then passes beneath the heating coils 6 which apply radiant heat to the paint film. The temperature of the web and the applied film is raised to approximately 165° F. and, after 30 equilibrium temperature has been reached in the web as it moves through the presetting device, radiant heat from the coils 6 is relied upon to maintain the desired temperature in the film and web. After the web 11 leaves the flat surface 35 of the coils 9, it rides upon a plate 24 secured at one end to the framework of the presetting device by an angle 25, the other end resting freely upon the coils 9. The decorated material then passes over a batten roll 26 through a vertically 40 extending dip 27 to an upper batten 28 from which it hangs in a festoon in the curing chamber 4 where sufficient heat is applied to properly set or 45 coagulate the vehicle, and, where a paint of my preferred type is employed, to effect conversion 45 of the resinoid with the oil of the vehicle to form a wear resistant surface which has good gloss characteristics and is stable, tough, flexible, and alkali-resistant.

It sometimes happens in printing machine operation that block chokes, shimming adjustments 50 and other causes require stopping the machine for a period of time greater than desirable for the application of heat to the decorated web in the presetting device. In order that the radiant heat applied to the surface may be rendered less intense, and further in order to avoid the application 55 of heat to the base web during such shut downs, means are provided whereby the radiant heaters may be moved away from the surface of the web a distance to render them sufficiently ineffective, and means are provided for injecting cooling fluid through the steam coils 9. In the embodiment illustrated, the frame-work 8 supporting the coils 6 is suspended from the shaft 60 29 by cables 30, two shafts 29 and four cables 30 being provided. Each shaft 29 is rotatable by a worm wheel 31 engaged by a worm operated by a handle 32, whereby the cables 30 are wound therearound and the radiant heaters 6 are elevated away from the surface of the decorated web. The connections from the source of steam 70 supply to the header 1 should preferably be made flexible to permit of such movement without the necessity of disjoining of pipes and fittings.

75 Any suitable connection may be made to the line

12 of the heating coils 9 for the passage of cooling water or other fluid therethrough. For example, a Y connection 33 may be used and a steam line 34 connected to one side thereof and a water line 35 connected to the other side. 5 Valves should be provided in each of these lines to effect proper control.

An electrically heated presetting device may be conveniently formed along the same general lines as those disclosed in the drawing, radiant heating coils being substituted for the steam coils 6 and an electrically heated platen replacing the coil 9. The mechanism for elevating the coils 6 may then be dispensed with and a control switch provided to cut off the heating current in the 15 event of a shut down of the printing machine.

The presetting device could utilize heated air if the time period for presetting were long enough. Care should, of course, be taken to insure that 20 the velocity of the air coming into contact with the wet film is not so great as to cause rippling or deformation of the applied pattern.

The presetting device illustrated in the drawing has been found to operate very satisfactorily with floor covering paints, both of the pigment "bodied up" type and of the type in which a false body is created by gel particles, resinoid particles or anisotropic pigment particles or combinations thereof. In the former type, the presetting device effects proper orientation of the 30 pigment and whatever minor amount of micelle formation which may be inherent in any oil paint film, and in the latter type the device operates to effect rapid micelle formation and concomitant thickening and stiffening of the 35 film induced thereby.

While I have illustrated and described certain preferred embodiments of my invention, it will be understood that the invention is not so limited but may be otherwise embodied within 40 the scope of the following claims.

I claim:

1. In the method of printing, the steps consisting in applying a film to a base, said film including oil and a resinoid which is but difficultly 45 soluble in the oil, said film having a thixotropic body susceptible to rapid micelle formation when shearing forces cease to be applied, applying heat to said film accelerate micelle formation while maintaining the base in a substantially 50 horizontal plane with the film at rest thereon, moving the base with its applied film through an inclined path, and curing said film at a temperature sufficient to effect substantially complete conversion of the resinoid with the oil. 55

2. In the method of coating a web, the steps consisting in applying a film of coating material to a base, said coating material including a partially regenerated oil gel, applying heat to said film while disposed in a substantially horizontal plane to effect micelle formation of the gel particles and concomitant thickening of the film, passing said base through an inclined path, and curing the film. 60

3. In the method of coating a web, the steps 65 consisting in applying a film of coating material including an oil vehicle containing resinoid particles dispersed therein to a base, applying heat to the film while disposed in a substantially horizontal plane, passing said base through an inclined path, and curing the film at a temperature sufficient to effect substantial conversion of the resin with the oil. 70

4. In the method of coating a web, the steps 75 consisting in applying a film of coating material

including a heat bodied oil vehicle containing oil gel particles, resinoid particles and pigment particles in dispersed condition therein to a base, the pigment being present in an amount less than 5 34% by volume of the nonvolatile constituent of the coating material, applying heat to said film while disposed in a substantially horizontal plane to effect micelle formation of the various particles, passing the base through an inclined path, and 10 curing the film.

5. In the method of coating a web, the steps consisting in applying to a substantially nonabsorptive web a relatively heavy film of coating material including an oil vehicle with particles 15 dispersed therein in a metastable condition, said particles having the characteristic of micelle formation, and being selected from a group consisting of oil gel, resinoid and flocculant pigments, said film of coating material when applied being 20 of such character that running will occur if the web be disposed in a substantially vertical plane, applying heat to said film while the same is disposed in a substantially horizontal plane to effect a thinning of the vehicle and a general leveling 25 of the applied film, continuing the application of heat while so disposed to effect conversion of said particles into micelles with concomitant thickening of said film in an amount sufficient to prevent running when disposed in a substantially vertical plane, passing said web with said film disposed thereon through an inclined path, and thereafter curing the film.

6. In the method of coating a web, the steps 30 consisting in applying to a substantially nonabsorptive web a relatively heavy film of coating material including oil vehicle with particles dispersed therein in a metastable condition, said particles having the characteristic of micelle formation and being selected from the group consisting of oil gel, resinoid and flocculent pigments, said coating material containing not more than 35 about 34% by volume of the nonvolatile portion thereof of pigment and being of such character that when applied running will occur if the web be disposed in a substantially vertical plane, applying heat to said film while the same is disposed in a substantially horizontal plane to effect conversion of said particles into micelles with concomitant thickening of said film in an amount sufficient to prevent running when disposed in a substantially vertical plane, passing the web with the film disposed thereon through an inclined path and thereafter curing the film.

7. In the method of coating a web, the steps 40 consisting in applying to a substantially nonabsorptive web a film of thixotropic bodied paint in a plurality of design elements, said paint including an oil vehicle with particles dispersed therein in a metastable condition, said particles having the characteristic of micelle formation and being selected from a group consisting of oil gel, resinoid and flocculent pigments, said paint when applied being of such character that running will occur if the web be disposed in a substantially vertical plane, applying heat to said elements while disposed on the base web in a substantially horizontal plane to effect leveling of the elements to a substantially plane, continuous film prior to thickening thereof by thixotropic action, contin-

uing the application of heat while so disposed to effect conversion of said particles into micelles with concomitant thickening of said film in an amount sufficient to prevent running when disposed in a substantially vertical plane, passing said web with said film disposed thereon through an inclined path, and thereafter curing the film.

8. In the method of coating a web required to be moved in an inclined path, the steps consisting in applying to a substantially non-absorptive web 10 a relatively heavy film of coating material including an oil vehicle with particles dispersed therein in a metastable condition, said particles having the characteristic of micelle or aggregate formation, and being selected from a group consisting of oil gel, resinoid and flocculent pigments, disposing said web so that a low viscosity film will not run thereon, while in such position applying heat to the applied film in an amount sufficient to reduce the viscosity of the film to permit natural leveling of the same, thereafter while the web is disposed in substantially the same manner effecting substantial thickening of the film by the application of additional heat thereto, moving the web in an inclined path and thereafter curing the 20 film by the continued application of heat.

9. In the method of coating a web, the steps consisting of applying to a substantially nonabsorptive web a relatively heavy film of coating material including an oil vehicle with oil gel particles dispersed therein in a metastable condition, applying heat to said film while disposed in a substantially horizontal plane to effect micelle formation of the gel particles and concomitant thickening of the film, passing the web through an inclined path and thereafter curing the film.

10. In the method of coating a web required to be moved in an inclined path, the steps consisting in applying to a substantially non-absorptive web a relatively heavy film of coating material including a vehicle with oil gel particles having the characteristic of micelle or aggregate formation dispersed therein in a metastable condition, said particles resulting from the treatment of a heat-bodied oil gel with a regenerating agent and thinning with a compatible oil, applying heat to said film while disposed in a substantially horizontal plane to effect such micelle or aggregate formation of the oil gel particles and concomitant thickening of the film, passing the web through an inclined path and thereafter curing the film.

11. In the method of coating a web required to be moved in an inclined path, the steps consisting in applying to a substantially non-absorptive web a relatively heavy film of coating material including a vehicle with resinoid particles having the characteristic of micelle or aggregate formation dispersed therein in a metastable condition, said particles resulting from the treatment of such resinoid with an oil in which the resinoid is not completely soluble and thinning the same with a thinning agent in which such resinoid is but difficultly soluble, applying heat to said film while disposed in a substantially horizontal plane to effect such micelle or aggregate formation of the resinoid particles and concomitant thickening of the film, passing the web through an inclined path and thereafter curing the film.

PHILIP H. PENNELL.